

June 23, 1931.

H. L. HALBACH

1,811,125

APPARATUS FOR DRAWING SHEET GLASS

Filed April 4 1928

2 Sheets-Sheet 1



Fig. 4.



INVENTOR

Howard L. Halbach  
by  
James C. Bradley  
atty

June 23, 1931.

H. L. HALBACH

1,811,125

APPARATUS FOR DRAWING SHEET GLASS

Filed April 4 1928 2 Sheets-Sheet 2



INVENTOR

Howard L. Halbach

by  
James T. Bracey  
Atty.

## UNITED STATES PATENT OFFICE

HOWARD L. HALBACH, OF CLARKSBURG, WEST VIRGINIA, ASSIGNOR TO PITTSBURGH PLATE GLASS COMPANY, A CORPORATION OF PENNSYLVANIA

## APPARATUS FOR DRAWING SHEET GLASS

Application filed April 4, 1928. Serial No. 267,240.

The invention relates to apparatus for drawing sheet glass. It has for its primary object the provision of means for preventing the sheet being drawn from thinning along lines inward from the side edges of the sheet in the use of the Slingluff drawing machine, such as disclosed in the Slingluff Patent No. 1,549,513. In the use of this apparatus, there is a tendency of the sheet to thin, as indicated at *a* in Fig. 4, which shows a horizontal section through the edge of a sheet produced on the Slingluff machine. This thinning of the sheet tends to increase the percentage of breakage and requires that a wider margin of the edge shall be trimmed off than would otherwise be the case. The present invention is designed to remedy this condition. One embodiment of the invention is illustrated in the accompanying drawings, wherein:

Figure 1 is a vertical section on the line I—I of Fig. 3. Fig. 2 is a horizontal section on the line II—II of Fig. 3. Fig. 3 is a vertical section on the line III—III of Fig. 1. And Fig. 4 is an enlarged horizontal section through the edge of a sheet produced on the Slingluff machine not employing the improvement to which the present invention relates.

Referring to the drawings, 1 is the end of a melting tank, preferably of the regenerator type; 2 is a drawing tank or kiln communicating with the melting tank; 3 is the lower end of a drawing apparatus provided with the pairs of driven rolls 4—4, 5—5, etc.; 6 is the draw bar extending transversely of the bath beneath the line of generation of the sheet 7; and 8, 8 are coolers to which the invention particularly relates extending transversely of the bath on opposite sides of the glass sheet.

The coolers are similar so that a description of one will be sufficient for both. They are made of cast or sheet metal with an inlet pipe 9 at one end and an outlet pipe 10 at the other, such pipes being provided with the valves 11 for regulating the flow. These pipes preferably connect to the top of the cooler at its ends, as indicated in Fig. 3 and the cooling fluid pursues the path indicated by the arrows in the drawings. In order to

give additional thicknesses at the points *a*, *a*, at which points the sheet normally runs somewhat thinner, the projecting portions 12, 12 are provided on the cooler, such projecting portions having their faces lying closer to the glass than the surface of the cooler intermediate such portions, so that the cooling effect upon the sheet is greater adjacent the ends of such sheet. It has been found that the provision of these means thickens up the sheet at the thin portions *a*, *a*, so that the breakage is reduced and the sheet may be trimmed closer to the edge than would otherwise be the case.

What I claim is:

The combination with apparatus for drawing a glass sheet continuously from a body of molten glass, of a hollow metal cooler extending transversely of the bath adjacent such bath and the glass sheet and having a pair of opposing vertical faces with the face next to the face of the sheet substantially parallel thereto, and provided opposite the marginal portions of the sheet with enlargements whose faces also lie parallel to the sheet and closer to the sheet than does the face of the cooler intermediate the enlargements, and means for circulating a cooling liquid through the cooler.

In testimony whereof, I have hereunto subscribed my name this 30th day of March, 1928.

HOWARD L. HALBACH.

55

60

65

70

75

85

90

95

100